# EUROPEAN PATENT SPECIFICATION

(11) **EP 0 000 599 B1**
(45) Date of publication and mention of the grant of the patent: **02.02.1983**
(21) Application number: 78200084.8
(22) Date of filing: 07.07.1978
(51) Int. Cl.: G03G 17/04, C09B 23/00

(54) **Electrically photosensitive particles for photoelectrophoretic migration imaging processes**
Elektrophotosensible Teilchen für photoelektrophoretische Bilderzeugung
Particules électrophotosensibles pour des procédés de formation d'images par migration photoélectrophorétique

(30) Priority: 25.07.1977 US 818697; 24.04.1978 US 899186
(43) Date of publication of application: 07.02.1979
(73) Proprietor: EASTMAN KODAK COMPANY (a New Jersey corporation), Rochester, New York 14650 (US)
(72) Inventor: Webster, Frank Glenn, Rochester New York (US); Regan, Michael Thomas, Fairport New York (US); Rossi, Louis Joseph, Rochester New York (US)
(74) Representative: Delaire, Marc

## Description

This invention relates to electrography and particularly to electrically photosensitive particles for photoelectrophoretic migration imaging processes, called hereafter "electrophoretic migration imaging processes".

In the past, there has been extensive description in the patent and other technical literature of electrophoretic migration imaging processes. For example, a description of such processes may be found in U.S. Patents 2,758,939, 2,940,847, 3,100,426, 3,140,175, 3,143,508, 3,384,565, 3,384,488, 3,615,558, 3,384,566 and 3,383,993. In addition to the foregoing patent literature directed to conventional photoelectrophoretic migration imaging processes, another type of electrophoretic migration imaging process which advantageously provides for image reversal is described in U.S. Patent 3,976,485. This latter process has been termed photoimmobilized electrophoretic recording or PIER.

In general, each of the foregoing electrophoretic migration imaging processes typically employs a layer of electrostatic charge-bearing photoconductive particles, i.e. electrically photosensitive particles, positioned between two spaced electrodes, one of which may be transparent. To achieve image formation in these processes, the charge-bearing photosensitive particles positioned between the two spaced electrodes, are subjected to the influence of an electric field an imagewise exposed to activating radiation. As a result, the charge-bearing electrically photosensitive particles are caused to migrate to the surface of one or the other of the spaced electrodes and one obtains an image pattern on the surface of these electrodes. Typically, a negative image is formed on one electrode and a positive image is formed on the ooposite electrode. Image discrimination occurs in the various electrophoretic migration imaging processes as a result of a net change in charge polarity of either the exposed electrically photosensitive particles (in the case of conventional electrophoretic migration imaging) or the unexposed electrically photosensitive particles (in the case of the electrophoretic migration imaging process described in the above-noted U.S. 3,976,485). Thus the image formed on one electrode surface is composed ideally of electrically photosensitive particles of a negative charge and the image formed on the other electrode surface is composed ideally of electrically photosensitive particles having a positive charge.

In any case, regardless of the particular electrophoretic migration imaging process employed, it is apparent that an essential component of any such process is the electrically photosensitive particles. And, of course, to obtain an easy-to-read, visible image, it is important that these electrically photosensitive particles be colored, as well as electrically photosensitive. Accordingly, as is apparent from the technical literature regarding electrophoretic migration imaging processes, work has been carried on in the past and is continuing to find particles which possess both useful levels of electrical photosensitivity and which exhibit good colorant properties. Thus, for example, various types of electrically photosensitive materials are disclosed for use in electrophoretic migration imaging processes, for example, in U.S. Patents 2,758,939, 2,940,847, 3,384,488 and 3,615,558, French Patent 2,185,814, in Research Disclosure n° 150 - October 1976 -Article 15 029 Hampshire U.K. Methine compounds containing cyano groups are described as photoconductive particles in photoelectrophoretic imaging processes in article 15 028 - Research Disclosure n° 150, October 1976 and as a sensitiser for photoconductive particles in PEP processes in DE 2,532,306.

The art has generally selected useful electrically photosensitive or photoconductive particles for electrophoretic migration imaging from known classes of photoconductive materials which may be employed in conventional photoconductive elements, e.g., photoconductive plates, drums, or webs used in electrophotographic office-copier devices, as taught for example in U.S. Patents 2,758,939 and 2,940,847. Also, the phthalocyanine pigments described as a useful electrically photosensitive particles for electrophoretic imaging processes in U.S. Patent 3,615,558 have long been known to exhibit useful photoconductive properties.

The object of the invention is to extend the diversity of particles available as electrically photosensitive particles for use in electrophoretic migration imaging processes by resorting to materials which, to the applicant's knowledge, have not been previously identified as photoconductors.

In accordance with the invention, electrically photosensitive particles for electrophoretic migration imaging processes, comprise a compound having the following formulas: or wherein:
m and n are zero, one or two;
L¹, L², L³, L⁴, L⁵, L⁶ and L⁷ represent hydrogen, cyano, alkyl, aralkyl, aryl, benzoyl or heterocyclyl, or in addition, any two of L¹, L² and L³ or any two of L⁴, L⁵, L⁶ and L may together represent the atoms needed to complete a carbocyclic ring having from 5-10 carbon atoms;
A¹ represents an alkyl or aryl substituted or unsubstituted aryl group or a substituted or unsubstituted heterocyclic nucleus;
A² represents a basic substituted or unsubstituted heterocyclic nucleus selected from the group consisting of: an imidazole; a 3H-indole; a thiazole; a benzothiazole; a naphthothiazole; a thianaphtheno-7',6', 4, 5-thiazole; an oxazole, a benzoxazole; a naphthoxazole; a selenazole; a benzoselenazole, a naphthoselenazole; a thiazoline; a 2-quinoline; a 4-quinoline; a 1-isoquinoline; a benzimidazole; a 2-pyridine; a 4-pyridine; a pyrrolo[1,2-a]pyridine; and an acenaphthothiazole;
B¹ and 8² represent cyano, carboxy, alkoxycarbonyl, aryloxycarbonyl, acyl, nitro.

In the above mentioned formulas, representatives of substituent A are an alkyl or aryl substituted or unsubstituted aryl (e.g. phenyl, naphthyl, anthryl) or a substituted or unsubstituted heterocyclic nucleus such as thiophene, benzo[b]thiophene, naphtho[2,3-b]thiophene, furan, isobenzofuran, chromene, pyran, xanthene, pyrrole, 2H-pyrrole, pyrazole, indolizine, indoline, indole, 3H-indole, indazole, carbazole, pyrimidine, isothiazole, isoxazole, furazan, chroman, isochroman, 1,2,3,4-tetrahydroquinoline; 4H-pyrrolo[3,2,1-ijlquinoline; 1,2-dihydro-4H-pyrrolo[3,2,1-ij]quinoline; 1,2,5,6-tetrahydro-4H-pyrrolo[3,2,1-ij]quinoline; 1H,5H-benzo[ijlquinolizine; 2,3-dihydro-1H,5H-benzo[ij]quino- lizine; 2,3,6,7-tetrahydro-1H, 5H-benzo[ij]quinolizine, 10, 11-dihydro-9H-benzo[a]xanthen-8-yl; 6,7-dihydro-5H-benzo[b]pyran-7-yl or pyrrolo[2,1-b]benzothiazole.

Representatives of substituent A are basic substituted or unsubstituted heterocyclic nuclei. Representative of such nuclei include:
a) an imidazole nucleus, such as imidazole and 4-phenylimidazole;
b) a 3H-indole nucleus such as 3H-indole, 3,3-dimethyl-3H-indole and 3,3,5-trimethyl-3H-indole;
c) a thiazole nucleus such as thiazole, 4-methylthiazole, 4-phenylthiazole, 5-methylthiazole, 5-phenylthiazole; 4,5-dimethylthiazole; 4,5-diphenylthiazole, and 4-(2-thienyl)thiazole;
d) a benzothiazole nucleus such as benzothiazole, 4-chlorobenzothiazole, 5-chlorobenzothiazole, 6-chlorobenzothiazole, 7-chlorobenzothiazole, 4-methylbenzothiazole, 5-methylbenzothiazole, 6-methylbenzothiazole, 5-bromobenzothiazole, 6-bromobenzothiazole, 4-phenylbenzothiazole, 5-phenylbenzothiazole, 4-methoxybenzothiazole, 5-methoxybenzothiazole, 6-methoxybenzothiazole, 5-iodobenzothiazole, 6-iodobenzothiazole, 4-ethoxybenzothiazole, 5-ethoxybenzothiazole, tetrahydrobenzothiazole, 5,6-dimethoxybenzothiazole, 5,6-dioxymethylenebenzothiazole, 5-hydroxybenzothiazole, and 6-hydroxybenzothiazole;
e) a naphthothiazole nucleus such as naphtho [1,2-d]-thiazole; naphtho[2,1-d]diazole, naphtho[2,3-d]thiazole, 5-methoxynaphtho[2,1-d]thiazole, 5-ethoxynaphtho[2,1-d]thiazole, 8-methoxynaphtho[2,1-d]thiazole, and 7-methoxynaphtho[2,1-d]thiazole;
f) a thianaphtheno-7',6',4,5-thiazole nucleus such as 4'-methoxythianaphtheno-7',6',4,5-thiazole;
g) an oxazole nucleus such as 4-methyloxazole, 5-methyloxazole, 4-phenyloxazole, 4,5-diphenyloxazole; 4-ethyloxazole; 4,5-dimethyloxazole, and 5-phenyloxazole;
h) a benzoxazole nucleus such as benzoxazole, 5-chlorobenzoxazole, 5-methylbenzoxazole, 5-phenylbenzoxazole, 6-methylbenzoxazole, 5,6-dimethylbenzoxazole; 4,6-dimethylbenzoxazole; 5-methoxybenzoxazole; 5-ethoxybenzoxazole; 5-chlorobenzoxazole; 6-methoxybenzoxazole; 5-hydroxybenzoxazole, and 6-hydroxybenzoxazole;
i) a naphthoxazole nucleus such as naphtho[1,2]oxazole and naphtho[2,1]oxazole;
j) a selenazole nucleus such as 4-methylselenazole and 4-phenylselenazole;
k) a benzoselenazole nucleus such as benzoselenazole, 5-chlorobenzoselenazole, 5-methoxy- benzoselenazole, 5-hydroxybenzoselenazole, and tetrahydrobenzoselenazole;
I) a naphthoselenazole nucleus such as naphtho[1,2-d]selenazole and naphtho[2,1-d]selenazole;
m) a thiazoline nucleus such as thiazoline and 4-methylthiazoline;
n) a 2-quinoline nucleus such as quinoline, 3-methylquinoline, 5-methylquinoline, 7-methylquinoline, 8-methylquinoline, 6-chloroquinoline, 8-chloroquinoline, 6-methoxyquinoline, 6- ethoxyquinoline, 6-hydroxyquinoline, and 8-hydroxyquinoline;
o) a 4-quinoline nucleus such as quinoline, 6-methoxyquinoline, 7-methylquinoline and 8-methylquinoline;
p) a 1-isoquinoline nucleus such as isoquinoline and 3,4-dihydroisoquinoline;
q) a benzimidazole nucleus such as 1,3-diethylbenzimidazole and 1-ethyl-3-phenylbenzimidazole;
r) a 2-pyridine nucleus such as pyridine and 5-methylpyridine;
s) a 4-pyridine nucleus;
t) a pyrrolo[1,2-a]pyridine nucleus; and
u) an acenaphthothiazole nucleus.

Representatives of substituent B¹ and 8² are cyano, carboxy, alkoxycarbonyl, aryloxycarbonyl, nitro, acyl such as arylcarbonyl, alkylsulfonyl, sulfonyl, fluorosulfonyl, trifluoromethylsulfonyl, carbamoyl, arylcarbamoyl, alkylcarbamoyl or heteroyl groups such as furoyl or benzofuroyl.

Alkyl refers to groups of 1-20 carbon atoms such as methyl, ethyl, propyl, isopropyl, butyl, heptyl, dodecyl, octadecyl. Aryl refers to aromatic ring groups of 6-20 carbons such as phenyl, naphthyl, anthryl or to alkyl or aryl substituted aryl groups such as tolyl, ethylphenyl, biphenylyl. Aralkyl refers to aryl substituted alkyl groups such as benzyl, phenethyl. Carbocyclic ring refers to saturated cycloalkyl groups which may have alkyl, aryl or aralkyl substituents such as cyclopropyl, cyclopentyl, cyclohexyl, 5,5-dimethylcyclohexyl, or refers to cyclohexene, dihydronaphthalene and 1 H-indene.

The materials of the present invention are relatively insoluble in imaging dispersions but are unexpectedly soluble in certain polymer coated image receiving elements. This solubility in the polymer coatings of image receiving elements results in images having excellent color saturation, density and resolution.

In accordance with the preferred embodiment of the present invention, the electrically photosensitive particles which are useful in electrophoretic migration imaging processes comprise compounds having a structure according to formula I or II wherein:
L¹, L², L³, L⁴, L⁵, L⁶ and L⁷, which may be the same or different represent hydrogen, cyano, methyl, phenyl, benzoyl, 2-thienyl, benzofuryl, 2-oxo-2H-benzo[b]pyran-3-yl or any two of L¹, L² and L³, or L⁴, L⁵, L and L⁷, may represent the atoms needed to complete a nucleus selected from the group consisting of dihydronaphthalene, 1H-indene and cyclohexene;
A represents an aryl group or a nucleus selected from the group consisting of indole; 1,2,5,6-tetrahydro-4H-pyrrolo-[3,2,1-ij]quinoline; 2,3,6,7-tetrahydro-1H,5H-benzo[ij]quinolizine and pyrrolo[2,1-b]benzothiazole;
A² represents a substituted and unsubstituted nucleus selected from the group consisting of 3H-indole, naphthothiazole, benzimidazole, 2-pyridine, pyrrolo[1,2-a]pyridine, benzoxazole, benzoselenazole and acenaphthothiazole; and
B¹ and B² represent cyano, ethoxycarbonyl, naphthoyl, benzoyl, benzofuroyl and dihydroxy benzoyl.

In general the particles which comprise compounds of Formulas I and II and which have been found to be electrophotosensitive tend to exhibit a maximum absorption wavelength, A max, within the range of from 420 to 750 nm. A variety of different particles within the class defined by Formulas I and II have been tested and found to exhibit useful levels of electrical photosensitivity in electrophoretic migration imaging processes.

Examples of such particles are disclosed in Table I. In Table I, Et represents -C₂H₅ and represents phenyl. Compounds disclosed herein are also disclosed in, among others, U.S. Patents 2,538,009; 2,721,799; 2,860,891; 2,860,981 and 2,860,982.

In general, electrically photosensitive particles useful in electrophoretic migration imaging processes have an average particle size within the range of from 0.01 micrometres to 20 micrometres, preferably from 0.01 to 5 micrometres. Typically, these particles are colorants. These electrically photosensitive particles may also contain various non photosensitive materials such as electrically insulating polymers, charge control agents, various organic and inorganic fillters, as well as various additional dyes or pigments to change or enhance various colorant and physical properties of the electrically photosensitive particles. In addition, such electrically photosensitive particles may contain other photosensitive materials such as various sensitizing dyes and/or chemical sensitizers to alter or enhance their response characteristic to activating radiation.

When used in an electrophoretic migration imaging process described in the present invention, the electrically photosensitive particles mentioned in Table I are positioned between two or more spaced electrodes, one or both of which typically being transparent to radiation to which the electrically photosensitive particles are light sensitive i.e., activating radiation. The electrically photosensitive particles may be dispersed simply as a dry powder between two spaced electrodes and then subjected to an electrophoretic migration imaging operation such as that described in U.S. Patent 2,758,939. It is more typical to disperse the electrically photosensitive particles in an electrically insulating carrier, such as an electrically insulating liquid or an electrically insulating, liquefiable matrix, such as a heat- and/or solvent-softenable polymer or a thixotropic polymer. Typically, when one employs such a dispersion of electrically photosensitive particles and electrically insulating carrier between the spaced electrodes of an electrophoretic migration imaging system, it is conventional to employ from 0.05 part to 2.0 parts of electrically photosensitive particles for each 10 parts by weight of electrically insulating carrier.

The carrier can comprise an electrically insulating liquid such as decane, paraffin, "Sohio Odorless Solvent 3440" (a kerosene fraction marketed by the Standard Oil Company, Ohio), various isoparaffinic hydrocarbon liquids such as those sold under the trakemark "Isopar G" by Exxon Corporation and having a boiling point in the range of 145°C to 186°C, various halogenated hydrocarbons such as carbon tetrachloride, tirchloromonofluoromethane, various alkylated aromatic hydrocarbon liquids such as the alkylated benzenes, for example, xylenes, and other alkylated aromatic hydrocarbons such as are described in U.S. Patent 2,899,335. An example of one such useful alkylated aromatic hydrocarbon liquid which is commercially available is "Solvesso 100" made by Exxon Corporation. "Solvesso 100" has a boiling point in the range of 157°C to 177°C and is composed of 9 percent xylene, 16 percent other monoalkyl benzenes, 34 percent dialkyl benzenes, 37 percent trialkyl benzenes, and 4 percent aliphatics. Typically, whether solid or liquid at normal room temperatures, i.e., 22°C, the electrically insulating carrier material used in the present invention is a material having a resistivity greater than 10⁹ ohm-cm, preferably greater than 10¹² ohm-cm.

When the electrically photosensitive particles of the present invention are incorporated in a carrier, such as one of the above-described electrically insulating liquids, various other addenda may be incorporated in the resultant imaging suspension. For example, various charge control agents may be incorporated in such a suspension to improve the uniformity of charge polarity of the electrically photosensitive particles dispersed in the liquid suspension. Such charge control agents are well known in the field of liquid electrograpic deve!opers where they are employed for purposes substantially similar to that described herein. Thus, extensive discussion of the charge control agents herein is deemed unnecessary. These charge control agents are typically polymers incorporated by admixture thereof into the liquid carrier of the suspension. In addition, charge control agents often provide more stable suspensions, i.e., suspensions which exhibit substantially less settling out of the dispersed photosensitive particles.

Useful polymeric charge control agents comprise a copolymer having at least two different repeating units,
(a) one of said units being present in an amount of at least 0.5 x 10-⁴ moles/gram of said copolymer and being derived from monomers selected from the group consisting of metal salts of sulfo acrylates and methacrylates and metal salts of acrylic and methacrylic acids, and
(b) one of said repeating units being derived from monomers soluble in said carrier vehicle and being present in an amount sufficient to render said copolymer dispersible in said carrier.

Examples of such copolymer charge control agents are poly(vinyltoluene-co-lauryl methacrylate-co-lithium methacrylate-co-methacrylic acid), poly(styrene-co-lauryl methacrylate-co-lithium sulfoethyl methacrylate), poly(vinyltoluene-co-lauryl methacrylate-co-lithium methacrylate), poly(styrene-co- lauryl methacrylate-co-lithium methacrylate), poly(t-butylstyrene-co-lauryl methacrylate-co-lithium methacrylate), and poly(t-butylstyrene-co-lithium methacrylate).

In addition to the foregoing charge control agents, various polymeric binders such as various natural, semi-synthetic resins, may be dispersed or dissolved in the electrically insulating carrier to fix the final photosensitive particle image formed on one of the spaced electrodes used in electrophoretic migration imaging systems. The use of such fixing addenda is conventional and well known in the closely related art of liquid electrographic developers so that extended discussion thereof is unnecessary herein.

The accompanying drawing illustrates a typical apparatus which employs an electrophoretic migration imaging process in which electrically photosensitive particles of the invention can be used.

The drawing shows a transparent electrode 1 supported by two rubber drive rollers 10 capable of imparting a translating motion to electrode 1 in the direction of the arrow. Electrode 1 may be composed of a layer of optically transparent material, such as glass or an electrically insulating, transparent polymeric support such as polyethylene terephthalate, this layer or support being covered with an optically transparent, conductive layer such as tin oxide, indium oxide, nickel. Optionally, depending upon the particular type of electrophoretic migration imaging process desired, the surface of electrode 1 may bear a "dark charge exchange" material, such as a solid solution of an electrically insulating polymer and 2,4,7,trinitro-9-fluorenone as described in the above-described Groner U.S. Patent 3,976,485 issued August 24, 1976.

Spaced opposite electrode 1 and in pressure contact therewith is a second electrode 5, an idler roller which serves as a counter electrode to electrode 1 for producing the electric field used in the electrophoretic migration imaging process. Typically, electrode 5 has on the surface thereof a thin, electrically insulating layer 6. Electrode 5 is connected to one side of the power source 15 by switch 7. The opposite side of the power source 15 is connected to electrode 1 so that as an exposure takes place, switch 7 is closed and an electric field is applied to the electrically photosensitive particles 4 which are positioned between electrodes 1 and 5. Typically electrically photosensitive particles 4 are dispersed in an electrically insulating carrier such as described hereinabove.

The electrically photosensitive particles 4 may be positioned between electrodes 1 and 5 by applying the particles 4 to either or both of the surfaces of electrodes 1 and 5 prior to the imaging process or by injecting the electrically photosensitive particles 4 between electrodes 1 and 5 during the electrophoretic migration imaging process.

As shown in the drawing, exposure of electrically photosensitive particles 4 takes place by use of an exposure system consisting of light source 8, an original image 11 to be reproduced, such as a photographic transparency, a lens system 12, and any necessary or desirable radiation filters 13, such as color filters, whereby electrically photosensitive particles 4 are irradiated with a pattern of activating radiation corresponding to original image 11. Although the electrophoretic migration imaging system represented in the drawing shows electrode 1 to be transparent to activating radiation from light source 8, it is possible to irradiate electrically photosensitive particles 4 in the nip 21 between electrodes 1 and 5 without either of electrodes 1 or 5 being transparent. In such a system, although not shown in the drawing, the exposure source 8 and lens system 12 is arranged so that particles 4 are exposed in the nip or gap 21 between electrodes 1 and 5.

As shown in the drawing, electrode 5 is a roller electrode having a conductive core 14 connected to power source 15. The core is in turn covered with a layer of insulating material 6, for example, baryta paper. Insulating material 6 serves to prevent or at least substantially reduce the capability of electrically photosensitive particles 4 to undergo a radiation induced charge alteration upon interaction with electrode 5. Hence, the term "blocking electrode" may be used, as is conventional in the art of electrophoretic migration imaging, to refer to electrode 5.

Although electrode 5 is shown as a roller electrode and electrode 1 is shown as a flat plate electrode in the drawing, either or both of these electrodes may assume a variety of different shapes such as a web electrode, rotating drum electrode, plate electrode, as is well known in the field of electrophoretic migration imaging. In general, during a typical electrophoretic migration imaging process wherein electrically photosensitive particles 4 are dispersed in an electrically insulating, liquid carrier, electrodes 1 and 5 are spaced such that they are in pressure contact or very close to one another during the electrophoretic migration imaging process, e.g., less than 50 micrometres apart. However, where electrically photosensitive particles 4 are dispersed simply in an air gap between electrodes 1 and 5 or in a carrier such as a layer of heat-softenable or other liquefiable material coated as a separate layer on electrode 1 and/or 5, these electrodes may be spaced more than 50 micrometres apart during the imaging process.

The strength of the electric field applied between electrodes 1 and 5 during the electrophoretic migration imaging process of the present invention may vary considerably; however, it has generally been found that optimum image density and resolution are obtained by increasing the field strength to as high a level as possible without causing electrical breakdown of the carrier in the gap between the electrodes. For example, when electrically insulating liquids such as isoparaffinic hydrocarbons are used as the carrier in the imaging apparatus of the drawing, the applied voltage across electrodes 1 and 5 typically is within the range of from 100 volts to 4 kilovolts.

As explained hereinabove, an image is formed in electrophoretic migration imaging processes as the result of the combined action of activating radiation and electric field on the electrically photosensitive particles 4 disposed between electrodes 1 and 5 in the attached drawing. Typically, for best results, field application and exposure to activating radiation occur concurrently. However, as would be expected, by appropriate selection of various process parameters such as field strength, activating radiation intensity, incorporation of suitable light sensitive addenda in or together with the electrically photosensitive particles by incorporation of a persistent photoconductive material, it is possible to alter the timing of the exposure and field application so that one may use sequential exposure and field application rather than concurrent field application and exposure.

When disposed between electrodes 1 and 5 of the drawing, electrically photosensitive particles 4 exhibit an electrostatic charge polarity, either as a result of triboelectric interaction of the particles or as a result of the particles interacting with the carrier in which they are dispersed, for example, an electrically insulating liquid, such as occurs in conventional liquid electrographic developers composed of toner particles which acquire a charge upon being dispersed in an electrically insulating carrier liquid.

Image discrimination occurs in the electrophoretic migration imaging process of the present invention as a result of the combined application of electric field and activating radiation on the electrically photosensitive particles dispersed between electrodes 1 and 5 of the apparatus shown in the drawing. That is, in a typical imaging operation, upon application of an electric field between electrodes 1 and 5, the electrically photosensitive particles 4 are attracted in the dark to either electrodes 1 or 5, depending upon which of these electrodes has a polarity opposite to that of the original charge polarity acquired by the electrically photosensitive particles. And, upon imagewise exposing particles 4 to activating radiation, it is theorized that there occurs neutralization or reversal of the charge polarity associated with either the exposed or unexposed particles. In typical electrophoretic migration imaging processes wherein electrode 1 bears a conductive surface, the exposed, electrically photosensitive particles 4, upon coming into electrical contact with such conductive surface, undergo an alteration (usually a reversal) of their original charge polarity as a result of the combined application of electric field and activating radiation. Alternatively, in the case of photoimmobilized electrophoretic recording (PIER), wherein the surface of electrode 1 bears a dark charge exchange material as described by Groner in aforementioned U.S. Patent 3,976,485, one obtains reversal of the charge polarity of the unexposed particles, while maintaining the original charge polarity of the exposed electrically photosensitive particles, as these particles come into.electrical contact with the dark charge exchange surface of electrode 1. In any case, upon the application of electric field and activating radiation to electrically photosensitive particles 4 disposed between electrodes 1 and 5 of the apparatus shown in the drawing, one can effectively obtain image discrimination so that an image is formed by the electrically photosensitive particles which corresponds to the original pattern of activating radiation. Using the apparatus shown in the drawing, one obtains a visible image on the surface of electrode 1 and a complementary image on the surface of electrode 5.

Subsequent to the application of the electric field and imagewise exposure to activating radiation, the images which are formed on the surface of electrodes 1 and 5 of the apparatus shown in the drawing may be temporarily or permanently fixed to these electrodes or may be transferred to a final image receiving element. Fixing of the final particle image can be effected by various techniques, for example, by applying a resinous coating over the surface of the image bearing substrate. For example, if electrically photosensitive particles 4 are dispersed in a liquid carrier between electrodes 1 and 5, one may fix the image or images formed on the surface of electrodes 1 and 5 by incorporating a polymeric binder in the carrier liquid. Many such binders (which are well known for use in liquid electrophotographic liquid developers) are known to acquire a change polarity upon being admixed in a carrier liquid and therefore will, themselves, electrophoretically migrate to the surface of one or the other of the electrodes. Alternatively, a coating of a resinous binder (which has been admixed in the carrier liquid), may be formed on the surfaces of electrodes 1 and 5 upon evaporation of the liquid carrier.

The electrically photosensitive particles comprising compounds of Formulas I & II may be used to form monochrome images, or the particles may be admixed with other electrically photosensitive particles of proper color and photosensitivity and used to form polychrome images.

Many of the electrically photosensitive particles comprising compounds having formulas I or II have especially useful hues which make them particularly suited for use in polychrome electrophoretic migration imaging processes which employ a mixture of two or more differently colored electrically photosensitive particles. When such a mixture of multicolored electrically photosensitive particles is formed, for example, in an electrically insulating carrier liquid, this liquid mixture of particles exhibits a black coloration. Preferably, the specific cyan, magenta, and yellow particles selected for use in such a polychrome electrophoretic migration imaging process are chosen so that their spectral response curves do not appreciably overlap whereby color separation and subtractive multicolor image reproduction can be achieved.

The following examples illustrate the utility of electrically photosensitive particles comprising the compounds of formulas I and II in electrophoretic migration imaging processes.

### Examples 1-45

### Imaging Apparatus

An imaging apparatus was used in each of the following examples to carry out the electrophoretic migration imaging process described herein. This apparatus was a device of the type illustrated in the drawing. In this apparatus, a film base having a conductive coating of 0.1 optical density cermet (Cr SiO) served as electrode 1 and was in pressure contact with a 10 centimeter diameter aluminum roller 14 covered with dielectric paper coated with poly(vinyl butyral) resin which served as electrode 5. Electrode 1 was supported by two 2.8 cm. diameter rubber drive rollers 10 positioned beneath electrode 1 such that a 2.5 cm. opening symmetrical with the axis of the aluminum roller 14, existed to allow exposure of electrically photosensitive particles 4 to activating radiation. The original transparency 11 to be reproduced was taped to the back side of electrode 1.

The original transparency to be reproduced consisted of adjacent strips of clear (WO), red (W29), green (W61) and blue (W47B) registered tradename Kodak Wratten filters. The light source consisted of a projector with a 1000 watt Xenon Lamp. The light was modulated with an eleven step 0.3 neutral density step tablet. The residence time in exposure zone was 10 milliseconds. The log of the light intensity (Log I) was as follows:

The voltage between the electrodes 1 and 5 was 2 kV. Electrode 1 was negative polarity in the case where electrically photosensitive particles 4 carried a positive electrostatic charge, and electrode 1 was positive in the case where electrically photosensitive particles 4 were negatively charged. The translational speed of electrode 1 was 25 cm. per second. In the following examples, an image was formed on the surfaces of electrodes 1 and 5 after simultaneous application of light exposure and electric field to electrically photosensitive particles 4 admixed with a liquid carrier as described below to form a liquid imaging dispersion and which dispersion had been placed in nip 21 between the electrodes 1 and 5. If the compounds being evaluated for use as particles 4 possessed a useful level of electrical photosensitivity, one obtained a negative-appearing image reproduction of original 11 on electrode 5 and a complementary image on electrode 1.

### Imaging Dispersion Preparation

Imaging dispersions were prepared to evaluate each of the compounds in Table I as electrically photosensitive particles. The dispersions were prepared by first making a stock solution of the following components. The stock solution was prepared simply by combining the components.

«. Poly(vinyltoluene - co - lauryl methacrylate - co - lithiu methacrylate - co - methacrylic acid) (56/40/3.6/0.4)
^{**} Vinyltoluene-styrene copolymer

A 5 g aliquot of the stock solution was combined in a closed container with 0.045 g of the Table I compound to be tested and 12 g of stainless steel balls. The preparation was then milled for three hours on a paint shaker.

Each of the 45 compounds described in Table I was tested according to the just outlined procedures. Each of the compounds was found to be electrophotosensitive as evidenced by obtaining a negative appearing image of the original on one electrode and a complementary image on the other electrode. Image quality was determined visually having regard to minimum and maximum densities, speed and color saturation.

### Examples 46-62

Imaging dispersions containing the Table I compounds listed in Table II were prepared as in the previous Examples 1-45. Imaging was also carried out as in the previous examples except the polymeric coating on the paper covering aluminum roller 14 was either Polymer A and Polymer B as indicated in Table II.

A portion of the imaged polymer coated paper for each Table II compound was heated at 170°C for 15 seconds. The sample generally changed to a brighter hue when heated in the polymer coating. Reflection spectra were taken of both the unheated and heated samples using diffuse illumination. Results are reported in Table II.

## Claims

1. Electrically photosensitive particles for photoelectrophoretic migration imaging processes characterized in that they comprise a compound having the following formulas: or wherein:
m and n are zero, one or two;
L¹, L², L³, L⁴, L⁵, L⁶ and L⁷ represent hydrogen, cyano, alkyl, aralkyl, aryl, benzoyl or heterocyclyl, or in addition, any two of L¹, L² and L³ or any two of L⁴, L⁵, L⁶ and L⁷ may together represent the atoms needed to complete a carbocyclic ring having from 5-10 carbon atoms;
A¹ represents an alkyl or aryl substituted or unsubstituted aryl group or a substituted or unsubstituted heterocyclic nucleus;
A² represents a basic substituted or unsubstituted heterocyclic nucleus selected from the group consisting of: an imidazole; a 3H-indole; a thiazole; a benzothiazole, a naphthothiazole; a thianaphtheno-7',6'-4,5-thiazole; an oxazole; a benzoxoazole; a naphthoxazole; a selenazole; a benzoselenazole; a naphthoselenazole; a thiazoline, a 2-quinoline; a 4-quinoline, a 1-isoquinoline; a benzimidazole; a 2-pyridine; a 4-pyridine; a pyrrolo[1,2-a]pyridine; and an acenaphthothiazole;
B¹ and B² represent cyano, carboxy, alkoxycarbonyl, aryloxycarbonyl, acyl, nitro provided that in the definitions above, an alkyl group has 1-20 carbon atoms and an aryl group has 6-20 carbon atoms.

2. Electrically photosensitive particles according to Claim 1 wherein A¹ is a nucleus selected from the group consisting of thiophene, benzo[b]thiophene, naphthoi2,3-b]thiophene, furan, isobenzofuran, chromene, pyran, xanthene, pyrrole, 2H-pyrrole, pyrazole, indolizine, indoline, indole, 3H-indole, indazole, carbazole, pyrimidine, isothiazole, isoxazole, furazan, chroman, isochroman, 1,2,3,4-tetrahydroquinoline, 4H-pyrrolo[3,2,1-ij]quinoline, 1,2-dihydro-4H-pyrrolo[3,2,1-ij]quinoline; 1,2,5,6-tetrahydro - 4H - pyrrolo[3,2,1 - ij]quinoline; 1H,5H - benzo[ij]quinolizine; 2,3 - dihydro - 1H,5H - benzo[ij]quinolizine; and 2,3,6,7 - tetrahydro - 1 H,5H - benzo[ij]quinolizine, 10,11 - dihydro - 9H - benzo[a]xanthen-8-yl; 6,7-dihydro-5H-benzo[b]pyran-7-yl and pyrrolo[2,7-b]benzothiazole.

3. Electrically photosensitive particles according to Claim 1 wherein A¹ represents a substituted or unsubstituted nucleus selected from the group consisting of indole; 1,2,5,6-tetrahydro-4H-pyrrolo[3,2,1-ij]quinoline; 2,3,6,7-tetrahydro-1H,5H-benzo[ij]quinolizine, and pyrrolo[2,1-b]benzothiazole;
A² represents a substituted and unsubstituted nucleus selected from the group consisting of 3H-indole; naphthothiazole; benzimidazole; 2-pyridine; pyrrolo[1,2-a]pyridine; benzoxazole; benzoselenazole; and acenaphthothiazole;
L¹, L², L³, L⁴, L⁵, L⁶ and L⁷ are the same or different and represent hydrogen, cyano, methyl, phenyl, benzoyl, 2-thienyl, benzofuryl, and 2-oxo-2H-benzo[b]pyran-3-yl or any two of L¹, L² and L³, or L⁴, L⁵, L⁶ and L⁷ represent the atoms needed to complete a nucleus selected from the group consisting of dihydronaphthalene, 1 H-indene and cyclohexene; and
B¹ and B² represent cyano, ethoxy carbonyl, naphthoyl, benzoyl, furoyl, benzofuroyl, or dihydroxy benzoyl.

4. Electrically photosensitive particles according to Claim 1 characterized in that they comprise a compound having formula II selected from the following group:

5. Electrically photosensitive particles according to claim 1, characterized in that they comprise the following compound having formula I.

## Patentansprüche

1. Elektrisch photosensitive Teilchen für photoelektrophoretische Bildherstellungsverfahren, dadurch gekennzeichnet, daß sie eine Verbindung der folgenden Formeln: oder worin bedeuten:
m und n = null, eins oder zwei;
L¹, L², L³, L⁴, L⁵, L⁶ und L⁷ Wasserstoff, Cyano, Alkyl, Aralkyl, Aryl, Benzoyl oder Heterocyclyl oder außerdem beliebige zwei von L¹, L² und L³ oder beliebige zwei von L⁴, L⁵, L⁶ und L⁷ gemeinsam die zur Vervollständigung eines carbocyclischen Ringes mit 5 bis 10 Kohlenstoffatomen erforderlichen Atome;
A¹ eine durch eine Alkyl- oder Arylgruppe substituierte oder unsubstituierte Arylgruppe oder ein substituierter oder unsubstituierter heterocyclischer Kern;
A² einen basischen substituierten oder unsubstituierten heterocyclischen Kern bestehend aus: einem Imidazol; einem 3H-Indol; einem Thiazol; einem Benzothiazol; einem Naphthothiazol; einem Thianaphtheno-7',6'-4,5-thiazol; einem Oxazol; einem Benzoxazol; einem Naphthoxazol; einem Selenazol; einem Benzoselenazol; einem Naphthoselenazol; einem Thiazolin; einem 2-Chinolin; einem 4-Chinolin; einem 1-Isochinolin; einem Benzimidazol; einem 2-Pyridin; einem 4-Pyridin; einem Pyrrolo[1,2-a]pyridin oder einem Acenaphthothiazol;
B¹ und B² Cyano-, Carboxy-, Alkoxycarbonyl-, Aryloxycarbonyl-, Acyl- oder Nitrogruppen, - vorausgesetzt, daß in den obigen Definitionen eine Alkylgruppe 1 bis 20 Kohlenstoffatome und eine Arylgruppe 6 bis 20 Kohlenstoffatome aufweist
enthalten oder daraus bestehen.

2. Elektrisch photosensitive Teilchen nach Anspruch 1, worin
A¹ ein Kern aus der Gruppe: Thiophen, Benzo[b]thiophen, Naphtho[2,3-b]thiophen, Furan, Isobenzofuran, Chromen, Pyran, Xanthen, Pyrrol, 2H-Pyrrol, Pyrazol, Indolizin, Indolin, Indol, 3H-Indol, Indazol, Carbazol, Pyrimidin, Isothiazol, Isoxazol, Furazan, Chroman, Isochroman, 1,2,3,4-Tetrahydrochinolin, 4H - Pyrrolo[3,2, 1 - ij]chinolin, 1,2 - Dihydro - 4H - pyrrolo[3,2, 1 - ij]chinolin; 1,2,5,6 - Tetrahydro - 4H - pyrrolo[3,2,1-ij]chinolin; 1 H,5H-Benzo[ij]chinolizin; 2,3-Dihydro-1 H,5H-benzo[ij]chinolizin und 2,3,6,7-Tetrahydro-1 H,5H-benzo[ij]chinolizin, 10,1 1-Dihydro-9H-benzo[a]xanthen-8-yl; 6,7-Dihydro-5H-benzo-[b]pyran-7-yl und Pyrrolo[2,1-b]benzothiazol
ist.

3. Elektrisch photosensitive Teilchen nach Anspruch 1, worin bedeuten:
A¹ einen substituierten oder unsubstituierten Kern aus der Gruppe: Indol; 1,2,5,6-Tetrahydro-4H-pyrrolo[3,2,1-ij]chinolin; 2,3,6,7-Tetrahydro-1 H,5H-benzo[ij]chinolizin und Pyrrolo[2,1-b]benzothiazol;
A² einen substituierten oder unsubstituierten Kern aus der Gruppe: 3H-Indol; Naphthothiazol; Benzimidazol; 2-Pyridin; Pyrrolo[1,2-a]pyridin; Benzoxazol; Benzoselenazol und Acenaphthothiazol;
L¹, L², L³, L⁴, L⁵, L⁶ und L⁷, die gleich oder verschieden sein können, Wasserstoff, Cyano, Methyl, Phenyl, Benzoyl, 2-Thienyl, Benzofuryl und 2-Oxo-2H-benzo[b]pyran-3-yl oder beliebige zwei von L¹, L² und L³ oder L⁴, L⁵, L⁶ und L⁷ die Atome, die zur Vervollständigung eines Kernes bestehend aus Dihydronaphthalin, 1H-Inden und Cyclohexen erforderlich sind und
B¹ und B² Cyano, Äthoxycarbonyl, Naphthoyl, Benzoyl, Furoyl, Benzofuroyl oder Dihydroxybenzoyl.

4. Elektrisch photosensitive Teilchen nach Anspruch 1, dadurch gekennzeichnet, daß sie eine Verbindung aufweisen, die eine Formel II aus der folgenden Gruppe von Formeln hat:

5. Elektrisch photosensitive Teilchen nach Anspruch 1, dadurch gekennzeichnet, daß sie die folgende Verbindung der Formel I aufweisen

## Revendications

1. Particules électrophotosensibles utilisables dans des procédés de formation d'images par migration photoélectrophorétique caractérisées en ce qu'elles comprennent un composé de formule: ou où m et n sont égaux à 0,1 ou 2;
L¹, L², L³, L⁴, L⁵, L⁶ et L⁷ représentent un atome d'hydrogène, des radicaux cyano, alkyle, aralkyle, aryle, benzoyle ou hétérocyclyle ou, en plus, deux quelconques des symboles L¹, L² et L³ ou deux quelconques des symboles L⁴, L⁵, L⁶ et L⁷ représentent ensemble les atomes nécessaires pour compléter un noyau carbocyclique de 5 à 10 atomes de carbone;
A¹ représente un groupe aryle substitué par un groupe alkyle ou aryle, un groupe aryle non substitué ou un noyau hétérocyclique substitué ou non;
A² représente un noyau basique hétérocyclique substitué ou non choisi dans le groupe formé par les noyaux imidazole, 3H-indole, thiazole, benzothiazole, naphthothiazole, thianaphténo-7',6',4,5-thiazole, oxazole, benzoxazole, naphtoxazole, sélénazole, benzosélénazole, naphtosélénazole, thiazoline, 2-quinoléine, 4-quinoléine, 1-isoquinoléine, benzimidazole, 2-pyridine, 4-pyridine, pyrrolo-[1,2-a]pyridine et acénaphtothiazole;
B¹ et B² représentent des radicaux cyano, carboxy, alkoxycarbonyle, aryloxycarbonyle, acyle, nitro; à condition que, dans les définitions précédentes, un groupe alkyle ait de 1 à 20 atomes de carbone et un groupe aryle ait de 6 à 20 atomes de carbone.

2. Particules électrophotosensibles conforme à la revendication 1, caractérisées en ce que A¹ représente un noyau choisi dans le groupe formé par les noyaux thiophène; benzo[b]thiophène; naphto[2,3-b]thiophène; furane; isobenzofurane; chromène; pyrane; xanthène; pyrrole; 2H-pyrrole, pyrazole; indolizine; indoline; indole; 3H-indole; indazole; carbazole; pyrimidine; isothiazole; isoxazole; furazane; chromane; isochromane; 1,2,3,4-tétrahydroquinoléine; 4H-pyrrolo[3,2,1-ij]quinoléine; 1,2-dihydro-4H-pyrrolo[3,2,1-ij]quinoléine; 1,2,5,6-tétrahydro-4H-pyrrolo[3,2,1-ij]quinoléine; 1H,5H-benzo[ij]quinolizine; 2,3-dihydro-1 H,5H-benzo[ij]quinolizine, 2,3,6,7-tétrahydro-l H,5H-benzo[ij]quino- lizine, 10,11-dihydro-9H-benzo[a]xanthen-8-yle, 6,7-dihydro-5H-benzo[b]pyran-7-yle et pyrrolo-[2,1-b]benzothiazole.

3. Particules électrophotosensibles conforme à la revendication 1, caractérisées en ce que A¹ représente un noyau substitué ou non choisi dans le groupe formé par les noyaux indole; 1,2,5,6-tétrahydro-4H-pyrrolo[3,2,1-ij]-quinoléine; 2,3,6,7-tétrahydro-1H,5H-benzo[ij]-quinolizine et pyrrolo-[2,1-b]benzothiazole;
A² représente un noyau substitué ou non choisi dans le groupe formé par les noyaux 3H-indole, naphtothiazole, benzimidazole, 2-pyridine, pyrrolo[1,2-a]pyridine, benzoxazole, benzosélénazole et acénaphtothiazole;
L¹, L², L³, L⁴, L⁵, L⁶ et L⁷ sont identiques ou différentes et représentent un atome d'hydrogène, un radical cyano, méthyle, phényle, benzoyle, 2-thiényle, benzofuryle ou 2-oxo-2H-benzo[b]pyran-3-yle ou bien deux quelconques des symboles L¹, L² et L³ ou deux quelconques des symboles L⁴, L⁵, L⁶ et L⁷ représentent les atomes nécessaires pour compléter un noyau choisi dans le groupe formé par le dihydronaphtalène, le 1 H-indène et le cyclohexène et
B¹ et B² représentent un radical cyano, éthoxycarbonyle, naphtoyle, benzoyle, furoyle, benzofuroyle ou dihydroxybenzoyle.

4. Particules électrophotosensibles conformes à la revendication 1, caractérisées en ce qu'elles comprennent un composé de formule Il choisi dans le groupe formé par:

5. Particules électrophotosensibles conformes à la revendication 1, caractérisées en ce qu'elles comprennent le composé suivant de formule I:
